

## UNITED STATES PATENT OFFICE

2,096,905

LUBRICATING OIL OF HIGH OILINESS AND  
RESISTANCE TO OXIDATION

Eugene Lieber, Linden, N. J., assignor to Standard Oil Development Company, a corporation of Delaware

No Drawing. Application August 22, 1935,  
Serial No. 37,302

14 Claims. (Cl. 87—9)

The present invention relates to improved lubricating oils, especially to oils of higher resistance to oxidation and of high oiliness characteristics. The present invention will be fully understood from the following description.

Mineral and other lubricating oils often do not of themselves possess a higher resistance to oxidation nor a high degree of oiliness, and various materials have been suggested to improve the oil in respect to one or the other of these properties. It is frequently the case that improvement in one respect is detrimental in the other. In the present instance, a new class of lubricating oil improvers is disclosed which simultaneously works an improvement in the oil both in respect to resistance to oxidation and to its oiliness value.

The particular class of substances which has been discovered at this time comprises the esters which contain sulphur or its equivalents, selenium and tellurium directly attached to an aromatic ring. Sulphur may be combined with the rings as mercaptan, disulphide or monosulphide, that is to say, thioether is quite effective when utilized in any of these three forms. These groups will be included in the term sulpho-aromatic groups but it will be understood that equivalents of the sulfur atom are included.

The aromatic ring may be phenolic or of the condensed form such as naphthalene or anthracene and the alkylated aromatic rings may also be used. Hydroxyl or amino groups may be present on the ring without detrimentally affecting the value of the compounds. Often indeed it is found to be improved by their presence.

The aromatic sulpho-radical may be present in the alcoholic or the acidic portion of the ester molecule and more than one of these groups is often desirable. The alcoholic portion of the ester may be an aromatic alcohol or phenol or it may be an aliphatic radical containing a substituted sulpho-aromatic group. It may be monohydric or polyhydric as will be illustrated below.

The acidic portion of the ester molecule may contain the sulpho-aromatic group whether or not such a group is a part of the alcoholic radical. Mono or poly basic acids may be employed.

In order more explicitly to disclose the type of compounds which fall within the class disclosed above, the following formulae are given,

but it will be understood that these are merely illustrations and are in no way limitative.



The esters are for the most part freely soluble in lubricating oils, but only relatively small quantities are necessary for the present purposes. As little as .01% is sufficient to greatly reduce the rate of oxidation of the oil, but more is usually preferred, say from .5 to 1% or even 2% or 5% or more may be desired to obtain the greatest oiliness values.

*Experiment*

To an SAE 50 hydrocarbon lubricating oil is added .5% of an acetic acid ester of di-tertiary butyl diphenol sulphide. Runs were made on the oil blank sample which did not contain these substances and on the blend, using the Mougey machine and method as described on page 47 in the National Petroleum News of November 11, 1931.

10

| Oil                                                                                    | Weights carried                      |
|----------------------------------------------------------------------------------------|--------------------------------------|
| 15 Hydrocarbon oil (blank)-----                                                        | 18 to 19—Sheared at 125 lbs. torque. |
| Hydrocarbon containing .5% of acetic ester of di-tertiary butyl diphenol sulphide----- | 25—18.5 inch pounds.                 |

20

The oil blend was very stable in respect to oxidation. The blended and unblended samples were subjected to an oxidation test in which oxygen was bubbled through the sample in a continuous circulatory stream at a fixed rate while the sample was held at 200° C. The rate of oxygen absorption is determined at 15 minute intervals by noting the volume of the undissolved oxygen.

30

| Samples         | Oxidation rate at 200° C. cc. of O <sub>2</sub> absorbed /15 min. interval /10 cc. sample |
|-----------------|-------------------------------------------------------------------------------------------|
| Blank-----      | 103—213—107                                                                               |
| 35 Blended----- | 30—31—25—29                                                                               |

The present invention is not limited to any theory of the improving agents nor to any particular agent mentioned in the disclosure, but only to the following claims in which it is desired to claim all novelty inherent in the invention.

I claim:

1. An improved lubricant comprising a lubricating oil and a small quantity of an ester containing an element selected from the group of sulphur, selenium and tellurium directly connected to an aromatic ring.

2. An improved lubricant comprising a lubricating oil and a small quantity of an ester containing a sulphur atom directly connected to an aromatic group.

3. An improved lubricant comprising a lubricating oil and a small quantity of an ester containing a sulphur atom directly connected to an aromatic group and being a compound selected from the class consisting of aromatic disulphides, mercaptans and thio-ethers.

4. An improved lubricant comprising a mineral lubricating oil and a small quantity of an ester containing an aromatic-mercapto group.

5. An improved lubricant comprising a petroleum lubricating oil and a small quantity of an ester containing an esterified mercapto-phenolic compound.

6. An improved lubricant comprising a lubricating oil and a small quantity of an ester containing an esterified mercapto-phenol.

7. An improved lubricant comprising a hydrocarbon lubricating oil and a small quantity of an ester containing an aromatic disulphide group.

8. An improved lubricant comprising a lubricating oil and a small quantity of an esterified disulphide of a phenolic compound.

9. An improved lubricant comprising a lubricating oil and a small quantity of an esterified disulphide of a phenol.

10. An improved lubricant comprising a lubricating oil and a small quantity of an ester with an aromatic thio-ether group.

11. An improved lubricant comprising a lubricating oil and a small quantity of an esterified phenolic compound with a thio-ether group.

12. An improved lubricant comprising a lubricating oil and a small quantity of an esterified phenol containing a thio-ether group.

13. An improved lubricant comprising a lubricating oil and a small quantity of an esterified diphenol thio-ether.

14. An improved lubricant comprising a lubricating oil and a small quantity of esterified alkyl diphenol thio-ether.

EUGENE LIEBER.

45